



US010353307B2

(12) **United States Patent**  
Miyoshi et al.

(10) **Patent No.:** US 10,353,307 B2  
(45) **Date of Patent:** Jul. 16, 2019

(54) **BRIGHT TONER, METHOD FOR PRODUCING BRIGHT TONER, AND IMAGE-FORMING APPARATUS**

(71) Applicants: **KABUSHIKI KAISHA TOSHIBA**, Minato-ku, Tokyo (JP); **TOSHIBA TEC KABUSHIKI KAISHA**, Shinagawa-ku, Tokyo (JP)

(72) Inventors: **Maiko Miyoshi**, Izunokuni Shizuoka (JP); **Li Xu**, Mishima Shizuoka (JP); **Taishi Takano**, Shimizu Sunto Shizuoka (JP)

(73) Assignees: **KABUSHIKI KAISHA TOSHIBA**, Tokyo (JP); **TOSHIBA TEC KABUSHIKI KAISHA**, Tokyo (JP)

(\*) Notice: Subject to any disclaimer, the term of this patent is extended or adjusted under 35 U.S.C. 154(b) by 0 days.

(21) Appl. No.: **15/872,652**

(22) Filed: **Jan. 16, 2018**

(65) **Prior Publication Data**

US 2019/0018328 A1 Jan. 17, 2019

(30) **Foreign Application Priority Data**

Jul. 14, 2017 (JP) ..... 2017-138077

(51) **Int. Cl.**

**G03G 9/08** (2006.01)  
**G03G 15/06** (2006.01)  
**G03G 9/087** (2006.01)  
**G03G 15/00** (2006.01)

(52) **U.S. Cl.**

CPC ..... **G03G 9/0819** (2013.01); **G03G 9/0808** (2013.01); **G03G 9/08755** (2013.01); **G03G 15/06** (2013.01); **G03G 15/6585** (2013.01)

(58) **Field of Classification Search**

CPC ..... G03G 9/0819; G03G 9/09; G03G 9/0902; G03G 9/0926

See application file for complete search history.

(56)

**References Cited**

**U.S. PATENT DOCUMENTS**

2006/0057482 A1 \* 3/2006 Yuasa ..... G03G 9/08773  
430/108.2  
2007/0128537 A1 \* 6/2007 Ariyoshi ..... G03G 9/0804  
430/137.1  
2007/0160923 A1 \* 7/2007 Matsumoto ..... B08B 7/0021  
430/108.1  
2008/0248415 A1 \* 10/2008 Maezawa ..... G03G 9/081  
430/112  
2008/0311503 A1 \* 12/2008 Nagaoka ..... G03G 9/0804  
430/110.1  
2009/0011355 A1 \* 1/2009 Shibai ..... G03G 9/0804  
430/109.1  
2009/0011357 A1 \* 1/2009 Kawase ..... G03G 9/0819  
430/110.1  
2009/0020899 A1 \* 1/2009 Matsumoto ..... C08J 3/12  
264/9  
2009/0232557 A1 \* 9/2009 Kikawa ..... G03G 9/0819  
399/252  
2011/0318682 A1 \* 12/2011 Takahashi ..... G03G 9/0819  
430/105  
2013/0137030 A1 \* 5/2013 Sato ..... G03G 9/0819  
430/108.11  
2014/0087302 A1 \* 3/2014 Kim ..... G03G 9/131  
430/114  
2016/0054669 A1 \* 2/2016 Hori ..... G03G 9/0827  
399/223  
2016/0054670 A1 \* 2/2016 Urabe ..... G03G 9/0823  
430/105  
2016/0070190 A1 \* 3/2016 Ishikawa ..... G03G 9/0812  
430/105  
2016/0179021 A1 \* 6/2016 Mizuhata ..... G03G 9/0804  
430/110.1  
2017/0139337 A1 \* 5/2017 Kaneko ..... G03G 9/087  
2018/0224783 A1 \* 8/2018 Matsumura ..... G03G 15/2092

\* cited by examiner

*Primary Examiner* — Christopher D Rodee

(74) *Attorney, Agent, or Firm* — Foley & Lardner LLP

(57) **ABSTRACT**

Provided here are toners and image forming apparatus and methods for the formation of a bright image with excellent brightness and concealability. A bright toner according to an embodiment comprises a plurality of toner particles containing a bright pigment and a binder resin, and has a volume particle diameter distribution with a coefficient of variation CV of 0.26 or more.

**20 Claims, 3 Drawing Sheets**

FIG. 1



FIG. 2



FIG. 3



## 1

**BRIGHT TONER, METHOD FOR  
PRODUCING BRIGHT TONER, AND  
IMAGE-FORMING APPARATUS**

**CROSS-REFERENCE TO RELATED  
APPLICATIONS**

This application claims the benefit of priority from Japanese Patent Application No. 2017-138077, filed Jul. 14, 2017, the entire contents of which are incorporated herein by reference.

**FIELD**

Embodiments described herein relate to a bright toner, a method for producing a bright toner, and an image forming apparatus.

**BACKGROUND**

With the recent diversification of the printed matter, there is a demand for a toner containing a pigment having brightness such as metallic luster or pearly luster as a colorant.

**BRIEF DESCRIPTION OF THE DRAWINGS**

FIG. 1 is a cross-sectional view schematically showing an example of an image forming apparatus.

FIG. 2 is a vertical cross-sectional view showing a structure of an image forming station.

FIG. 3 is a block diagram showing a schematic structure of a control system.

**DETAILED DESCRIPTION**

Hereinafter, embodiments will be described with reference to the drawings. Incidentally, components having the same or similar functions are denoted by the same reference numerals, and repetitive explanations will be omitted.

An object of some embodiments described herein is to provide toners and image forming apparatus and methods for the formation of a bright image with excellent brightness and concealability.

A bright toner according to a first embodiment includes a plurality of toner particles containing a bright pigment and a binder resin, and having a volume particle diameter distribution with a coefficient of variation CV of 0.26 or more.

A method for producing a bright toner according to a second embodiment includes mixing a first toner which includes a plurality of first toner particles containing a first bright pigment and a first binder resin, and a second toner which includes a plurality of second toner particles containing a second bright pigment and a second binder resin, and has a volume average particle diameter, the ratio of which to the volume average particle diameter of the first toner is 1.10 or more in such amounts that the ratio of the amount of the second toner to the total amount of the first toner and the second toner is within the range of 30 to 90 mass %.

An image forming apparatus according to a third embodiment includes a photoconductor, a charger which charges the photoconductor, an optical unit which irradiates the photoconductor with light, thereby forming an electrostatic latent image, a developing device which supplies a bright toner including a plurality of toner particles containing a bright pigment and a binder resin and having a volume particle diameter distribution with a coefficient of variation CV of

## 2

0.26 or more to the photoconductor, thereby forming a toner image corresponding to the electrostatic latent image, and a transfer device which directly or indirectly transfers the toner image onto a recording medium from the photoconductor.

Examples of the bright pigment described herein include mica coated with a metal oxide and an aluminum pigment. In some embodiments, the bright pigment can have a flat plate shape, and the principal plane thereof can function as a reflective surface. Therefore, as the particle diameter of the bright pigment becomes larger, the bright pigment can exhibit metallic luster or pearly luster more strongly.

<<Image Forming Apparatus>>

An image forming apparatus according to an embodiment includes a photoconductor, a charger which charges the photoconductor, an optical unit which irradiates the photoconductor with light, thereby forming an electrostatic latent image, a developing device which supplies a bright toner including a plurality of toner particles containing a bright pigment and a binder resin and having a volume particle diameter distribution with a coefficient of variation CV of 0.26 or more to the photoconductor, thereby forming a toner image corresponding to the electrostatic latent image, and a transfer device which directly or indirectly transfers the toner image onto a recording medium from the photoconductor.

One example of the image forming apparatus will be described with reference to FIGS. 1 to 3.

FIG. 1 is a vertical cross-sectional view schematically showing the overall structure of the image forming apparatus according to one example. FIG. 2 is a cross-sectional view schematically showing a structure of an image forming station included in the image forming apparatus shown in FIG. 1. FIG. 3 is a block diagram showing a schematic structure of a control system of the image forming apparatus shown in FIG. 1.

An image forming apparatus 1 shown in FIG. 1 is a color multi-functional peripheral (MFP). The image forming apparatus 1 includes a housing 2, a printer section 3 placed in the housing 2, and a scanner section 4 placed on the upper surface of the housing 2.

The printer section 3 forms an image on a recording medium, here, on a sheet such as a paper or a resin film by electrophotography. The printer section 3 includes a paper feed section 10, an optical unit 20, an image forming section 50, a fixing section 70, a carrying section 80, an image information input section 100, and a control section 200.

The paper feed section 10 includes a plurality of paper feed cassettes 11 and a plurality of pickup rollers 12. Each of these paper feed cassettes 11 stores stacked sheets. The pickup roller 12 feeds a sheet P which is the top layer among the sheets stored in the paper feed cassette 11 to the image forming section 50.

The optical unit 20 exposes the below-mentioned photoconductors 61Y, 61M, 61C, and 61K to light, and electrostatic latent images are formed on the surfaces thereof. As the optical unit 20, for example, a laser or a light-emitting diode (LED) can be used.

The image forming section 50 includes an intermediate transfer belt 51, a plurality of rollers 52, a secondary transfer roller 54, a backup roller 55, image forming stations 60Y, 60M, 60C, and 60K, hoppers 66Y, 66M, 66C, and 66K, and toner cartridges 67Y, 67M, 67C, and 67K. The below-mentioned primary transfer rollers 64Y, 64M, 64C, and 64K, the intermediate transfer belt 51, the plurality of rollers 52, the secondary transfer roller 54, and the backup roller 55 constitute a transfer device.

The intermediate transfer belt 51 temporarily holds toner images formed by the image forming stations 60Y, 60M, 60C, and 60K. The plurality of rollers 52 provide a tension to the intermediate transfer belt 51. The secondary transfer roller 54 drives the intermediate transfer belt 51. Between the secondary transfer roller 54 and the backup roller 55, a part of the intermediate transfer belt 51 is interposed. The backup roller 55 transfers the toner image formed on the intermediate transfer belt 51 to the sheet P along with the secondary transfer roller 54.

The image forming stations 60Y, 60M, 60C, and 60K have the same structure. That is, as shown in FIG. 2, the image forming station 60Y includes the photoconductor 61Y, a charger 62Y, a developing device 63Y, the primary transfer roller 64Y, and a cleaning unit 65Y. The image forming station 60M includes the photoconductor 61M, a charger 62M, a developing device 63M, the primary transfer roller 64M, and a cleaning unit 65M. The image forming station 60C includes the photoconductor 61C, a charger 62C, a developing device 63C, the primary transfer roller 64C, and a cleaning unit 65C. The image forming station 60K includes the photoconductor 61K, a charger 62K, a developing device 63K, the primary transfer roller 64K, and a cleaning unit 65K.

Here, the photoconductors 61Y, 61M, 61C, and 61K are photoconductive drums. The photoconductors 61Y, 61M, 61C, and 61K may be photoconductive belts. Further, here, for the image forming stations 60Y, 60M, 60C, and 60K, the photoconductors 61Y, 61M, 61C, and 61K are provided, respectively, however, one photoconductor may be provided for the image forming stations 60Y, 60M, 60C, and 60K.

The chargers 62Y, 62M, 62C, and 62K impart a negative charge to the photoconductors 61Y, 61M, 61C, and 61K, respectively, and uniformly charge the surfaces thereof with negative static electricity.

The developing device 63Y includes a developing container 631Y, developer mixers 632Y and 633Y, and a developing roller 635Y. The developer mixers 632Y and 633Y stir the developer in the developing container 631Y and also supply this developer to the developing roller 635Y. The developing roller 635Y supplies this developer to the photoconductor 61Y.

The developing device 63M includes a developing container 631M, developer mixers 632M and 633M, and a developing roller 635M. The developer mixers 632M and 633M stir the developer in the developing container 631M and also supply this developer to the developing roller 635M. The developing roller 635M supplies this developer to the photoconductor 61M.

The developing device 63C includes a developing container 631C, developer mixers 632C and 633C, and a developing roller 635C. The developer mixers 632C and 633C stir the developer in the developing container 631C and also supply this developer to the developing roller 635C. The developing roller 635C supplies this developer to the photoconductor 61C.

The developing device 63K includes a developing container 631K, developer mixers 632K and 633K, and a developing roller 635K. The developer mixers 632K and 633K stir the developer in the developing container 631K and also supply this developer to the developing roller 635K. The developing roller 635K supplies this developer to the photoconductor 61K.

The developing devices 63Y, 63M, 63C, and 63K supply a developer to the photoconductors 61Y, 61M, 61C, and 61K, respectively, to form toner images corresponding to the electrostatic latent images. One to three developing devices

among the developing devices 63Y, 63M, 63C, and 63K can be omitted. Further, the image forming section 50 may further include one or more other developing devices in addition to the developing devices 63Y, 63M, 63C, and 63K. The developer and the toner will be described in detail later.

The primary transfer rollers 64Y, 64M, 64C, and 64K transfer the toner images on the photoconductors 61Y, 61M, 61C, and 61K to the intermediate transfer belt 51, respectively.

10 The cleaning units 65Y, 65M, 65C, and 65K clean a residue on the photoconductors 61Y, 61M, 61C, and 61K, respectively.

The hoppers 66Y, 66M, 66C, and 66K are placed above the developing devices 63Y, 63M, 63C, and 63K, respectively. The hoppers 66Y, 66M, 66C, and 66K replenish the developer to the developing devices 63Y, 63M, 63C, and 63K, respectively.

The toner cartridges 67Y, 67M, 67C, and 67K are detachably placed above the hoppers 66Y, 66M, 66C, and 66K, respectively. The toner cartridges 67Y, 67M, 67C, and 67K include toner cartridge bodies 671Y, 671M, 671C, and 671K, respectively. Each of the toner cartridge bodies 671Y, 671M, 671C, and 671K is one example of the container and stores the developer. The toner cartridges 67Y, 67M, 67C, and 67K supply the developer to the hoppers 66Y, 66M, 66C, and 66K, respectively.

The fixing section 70 includes a heating roller, a pressure member, a pad, a spring, and a stopper (all not shown). The fixing section 70 is placed at a position on a path where the carrying section 80 carries the sheet P and between the secondary transfer roller 54 and a paper discharge roller 83.

The carrying section 80 includes a resist roller 81, a carrying roller 82, a paper discharge roller 83, and a paper discharge tray 84. The resist roller 81 starts the carrying of the sheet P fed from the pickup roller 12 to the image forming section 50 at a predetermined timing. The carrying roller 82 carries the sheet P fed from the resist roller 81 so that the sheet P passes between the backup roller 55 and the intermediate transfer belt 51, and thereafter passes through 35 the fixing section 70. The paper discharge roller 83 is located on a path where the sheet P is carried and immediately upstream of the position where the sheet P is discharged 40 outside the printer section 3 and carries the sheet P to the paper discharge tray 84. The paper discharge tray 84 is located on the upper surface of the printer section 3 and receives the discharged sheet P.

The image information input section 100 takes in the image information to be printed on the sheet P which is a recording medium from an external recording medium or a network. The image information input section 100 supplies this image information to the control section 200.

The control section 200 includes a memory section 210 and a processing section 220. The memory section 210 includes, for example, a primary memory device (for example, Random Access Memory (RAM)) and a secondary memory device (for example, Read Only Memory (ROM)). The processing section 220 includes a processor (for example, Central Processing Unit (CPU)). The secondary memory device stores, for example, a program to be interpreted and executed by the processor. The primary memory device primarily stores, for example, the image information supplied from the image information input section 100 or the like, the program stored by the secondary memory device, and data or the like generated by the processing by the processor. The processor interprets and executes the program stored by the primary memory device. The control section 200 controls the operation of the paper feed section

10, the optical unit 20, the image forming section 50, the fixing section 70, the carrying section 80, etc. based on the image information supplied from the image information input section 100 or the like in this manner.

<<Developer>>

Next, the developer which can be used in the above-mentioned image forming apparatus 1 will be described.

In the image forming apparatus 1 described with reference to FIGS. 1 to 3, for example, a two-component developer containing a toner and a carrier can be used.

The carrier is not particularly limited, however, for example, a ferrite carrier can be used.

One of the toner cartridges 67Y, 67M, 67C, and 67K includes a bright toner described below as the toner. Here, as one example, it is assumed that the toner cartridge 67K includes the bright toner. That is, the bright toner is stored in the toner cartridge body 671K which is one example of the container.

The bright toner can be distributed alone. For example, the bright toner can be distributed by being stored in a container.

Alternatively, the bright toner may be mixed with a carrier. That is, the bright toner may be distributed in the form of a developer containing the bright toner and a carrier and stored in the container. In this case, according to one example, the container is the toner cartridge body 671K. That is, the bright toner may be distributed in the form of a toner cartridge. Alternatively, the container may be a container other than the toner cartridge body.

The volume particle diameter distribution of the bright toner has a coefficient of variation CV of 0.26 or more. Here, the "volume particle diameter distribution" means values obtained by particle size distribution measurement using an electrical sensing zone method (the Coulter Principle). Further, the "coefficient of variation CV" is a value calculated from the above-mentioned volume average particle diameter (average value) and the standard deviation of the volume particle diameter obtained by the above-mentioned particle size distribution measurement and means a value obtained according to the following formula 1. Incidentally, the "volume average particle diameter" means a 50% volume average particle diameter.

$$\text{Coefficient of variation } CV = \frac{\text{Standard deviation}}{\text{Average value}} \quad (\text{Formula 1})$$

When the coefficient of variation CV is too small, excellent brightness and excellent concealability cannot be achieved simultaneously. This coefficient of variation CV does not have an upper limit, however, according to one example, the coefficient of variation CV is 0.30 or less.

The volume average particle diameter of the bright toner is preferably within the range of 7.0 to 105.0  $\mu\text{m}$ , more preferably within the range of 16.0 to 17.7  $\mu\text{m}$ . When the volume average particle diameter is within the above range, particularly excellent performance with respect to both brightness and concealability can be achieved.

The toner particles included in the bright toner contain a bright pigment and a binder resin. Hereinafter, these components will be described.

(Binder Resin)

As the binder resin, for example, a polyester-based resin, a styrene-acrylic-based resin, a polyurethane-based resin, or an epoxy-based resin can be used.

As the polyester-based resin, for example, a polyester-based resin obtained using, as a raw material monomer, a dihydric or higher hydric alcohol component and a divalent

or higher valent carboxylic acid component such as a carboxylic acid, a carboxylic anhydride, or a carboxylic ester can be used.

As the divalent or higher valent carboxylic acid component, for example, an aromatic dicarboxylic acid such as terephthalic acid, phthalic acid, or isophthalic acid, or an aliphatic carboxylic acid such as fumaric acid, maleic acid, succinic acid, adipic acid, sebacic acid, glutaric acid, pimelic acid, oxalic acid, malonic acid, citraconic acid, or itaconic acid can be used.

As the dihydric or higher hydric alcohol component, for example, an aliphatic diol such as ethylene glycol, propylene glycol, 1,4-butanediol, 1,3-butanediol, 1,5-pentanediol, 1,6-hexanediol, neopentyl glycol, trimethylene glycol, trimethylolpropane, or pentaerythritol, an alicyclic diol such as 1,4-cyclohexanediol or 1,4-cyclohexanedimethanol, an ethylene oxide such as bisphenol A, or a propylene oxide adduct or the like can be used.

Further, the above-mentioned polyester components may be converted so as to have a crosslinked structure using a trivalent or higher valent carboxylic acid component or a trihydric or higher hydric alcohol component such as 1,2,4-benzenetricarboxylic acid (trimellitic acid) or glycerin. Further, as the binder resin, a mixture of two or more types of polyester resins having different compositions may be used.

The polyester-based resin may be crystalline or amorphous.

The glass transition temperature of the polyester-based resin is preferably within the range of 35° C. to 70° C., more preferably within the range of 40° C. to 65° C. When the glass transition temperature is too low, the storage stability of the toner may be deteriorated. When the glass transition temperature is too high, the low-temperature fixability may be deteriorated.

As the styrene-acrylic-based resin, for example, a polymer of a styrene, a copolymer of a styrene and a diene, or a copolymer of a styrene and an alkyl (meth)acrylate can be used.

The binder resin is not particularly limited, but is preferably a polyester-based resin. The polyester-based resin has a lower glass transition temperature than, for example, a styrene-based resin, and therefore, when the polyester-based resin is used as the binder resin, more excellent low-temperature fixability can be achieved.

(Bright Pigment)

The bright pigment is a pigment which has a flat plate shape with brightness such as metallic luster or pearly luster.

As the bright pigment, for example, a flaky powder composed of a metal such as aluminum, brass, bronze, nickel, stainless steel, or zinc, a coated flaky inorganic crystal substrate obtained by coating a flaky inorganic compound such as mica, barium sulfate, or a layered silicate with an inorganic oxide such as titanium oxide or yellow iron oxide, single crystal plate-like titanium oxide, a flaky powder composed of a basic carbonate, a flaky powder composed of bismuth oxychloride, a flaky powder composed of natural guanine, a flaky glass powder, or a metal-deposited flaky glass powder can be used.

The bright toner may contain bright pigments which exhibit brightness on different principles, but preferably contains only bright pigments which exhibit brightness on the same principle, and more preferably contains only bright pigments composed of the same material.

According to one example, the bright toner contains only pigments which exhibit metallic luster as the bright pig-

ments. In this case, the bright pigments are preferably composed of the same material.

According to another example, the bright toner contains only pigments which exhibit brightness by utilizing multiple reflection interference, for example, pigments which exhibit pearly luster as the bright pigments. In this case, the bright pigments are preferably composed of the same material, for example, all the bright pigments are composed of a coated flaky inorganic crystal substrate obtained by coating mica with an inorganic oxide.

The volume average particle diameter of the bright pigment is preferably within the range of 6 to 100  $\mu\text{m}$ , more preferably within the range of 6 to 50  $\mu\text{m}$ . When the volume average particle diameter of the bright pigment is too small, a sufficient decorative property may not be obtained. When the volume average particle diameter of the bright pigment is too large, it may be hard to control the development, transfer, or the like. When the volume average particle diameter of the bright pigment is within the above range, it is advantageous for obtaining particles which achieve a favorable decorative property and also facilitate the above-mentioned control.

According to one example, the volume particle size distribution of the bright pigment has a coefficient of variation CV in the range of 0.41 to 0.50. Further, the number particle size distribution of the bright pigment has a coefficient of variation CV in the range of 0.50 to 0.57. Here, the "number particle size distribution" means values obtained by measurement using an electrical sensing zone method.

As the bright pigment, a commercially available product may be used. As the commercially available product, for example, Iridin (registered trademark) 325 (Merck Corporation) or Iridin 305 (Merck Corporation) can be used.

The amount of the bright pigment is preferably within the range of 10 to 100 parts by mass with respect to 100 parts by mass of the binder resin. When the amount of the bright pigment is small, it is hard to achieve excellent brightness. When the amount of the bright pigment is large, a problem may occur in the fixability or the like.

<Release Agent>

The toner particles may further contain a release agent. As the release agent, for example, a low-molecular weight polyethylene, a low-molecular weight polypropylene, a polyolefin copolymer, an aliphatic hydrocarbon-based wax such as a polyolefin wax, a microcrystalline wax, a paraffin wax, or a Fischer-Tropsch wax, or a modified material thereof, an oxide of an aliphatic hydrocarbon-based wax such as a polyethylene oxide wax, or a block copolymer thereof, a vegetable wax such as candelilla wax, carnauba wax, Japan wax, jojoba wax, or rice wax, an animal wax such as bees wax, lanolin, or spermaceti wax, a mineral wax such as montan wax, ozokerite, ceresin, or petrolacum, a wax containing a fatty acid ester as a main component such as a montanic ester wax or a castor wax, or a wax obtained by partially or entirely deoxidizing a fatty acid ester such as a deoxidized carnauba wax can be used. The release agent may be omitted. When the release agent is used, the amount thereof is preferably within the range of 5 to 40 parts by mass, more preferably within the range of 10 to 20 parts by mass with respect to 100 parts by mass of the mother toner, that is, the toner particles.

<Charge Control Agent>

The toner particles may further contain a charge control agent. As the charge control agent, for example, a metal-containing azo compound can be used. The metal-containing azo compound is a complex or a complex salt in which the metal element is, for example, iron, cobalt, or chromium. As

the metal-containing azo compound, one type among these may be used alone or two or more types may be used. Further, as the charge control agent, for example, a metal-containing salicylic acid derivative compound can also be used. The metal-containing salicylic acid derivative compound is a complex or a complex salt in which the metal element is, for example, zirconium, zinc, chromium, or boron. As the metal-containing salicylic acid derivative compound, one type among these may be used alone or two or more types may be used. The charge control agent may be omitted. When the charge control agent is used, the amount thereof is preferably within the range of 0.01 to 5.00 parts by mass, more preferably within the range of 0.1 to 2 parts by mass with respect to 100 parts by mass of the mother toner. (External Additive)

The bright toner may further include an external additive carried on the surfaces of the toner particles. As the external additive, for example, inorganic fine particles can be used. As the inorganic fine particles, for example, silica, titania, alumina, strontium titanate, tin oxide, or the like can be used. As the inorganic fine particles, one type among these may be used alone or two or more types may be used. The further external addition of the inorganic fine particles to the toner particles is advantageous for adjusting the fluidity and chargeability of the toner. Further, as the inorganic fine particles, those surface-treated with a hydrophobizing agent are preferably used. By using the inorganic fine particles surface-treated with a hydrophobizing agent, more excellent environmental stability can be achieved. When the inorganic fine particles are used as the external additive, the amount thereof is preferably within the range of 0.1 to 10 parts by mass, more preferably within the range of 0.2 to 5 parts by mass with respect to 100 parts by mass of the mother toner.

The bright toner may further include resin fine particles with a size of 1  $\mu\text{m}$  or less carried on the surfaces of the toner particles.

The external additive may be omitted.

When the resin fine particles are used as the external additive, the amount thereof is preferably within the range of 0.01 to 5 parts by mass, more preferably within the range of 0.1 to 2 parts by mass with respect to 100 parts by mass of the mother toner.

<<Method for Producing Bright Toner>>

The bright toner of this embodiment is produced by, for example, the following method. That is, the bright toner can be produced by a method including mixing a first toner which includes a plurality of first toner particles containing a first bright pigment and a first binder resin, and a second toner which includes a plurality of second toner particles containing a second bright pigment and a second binder resin, and has a volume average particle diameter, the ratio of which to the volume average particle diameter of the first toner is 1.10 or more in such amounts that the ratio of the amount of the second toner to the total amount of the first toner and the second toner is within the range of 30 to 90 mass %.

Hereinafter, the first and second toners which can be used in the production of the bright toner will be described in detail.

<First Toner>

The volume average particle diameter of the first toner is preferably within the range of 6 to 100  $\mu\text{m}$ , more preferably within the range of 6 to 50  $\mu\text{m}$ , further more preferably within the range of 6 to 30  $\mu\text{m}$ . When the volume average particle diameter is too small, it is hard to form a bright image with excellent brightness. When the volume average

particle diameter is too large, it is hard to form a bright image with excellent concealability.

The volume average particle diameter of the toner refers to the 50% volume average particle diameter of the toner obtained by externally adding an external additive to the toner particles. However, the volume average particle diameter of the toner particles before the external additive is added, that is, a mother toner (or toner core particles) and the volume average particle diameter of the toner obtained by externally adding an external additive to the toner particles are substantially the same.

<Second Toner>

The second toner has a volume average particle diameter, the ratio of which to the volume average particle diameter of the first toner is 1.10 or more. This ratio is preferably within the range of 1.10 to 1.50, more preferably within the range of 1.20 to 1.50. When this ratio is too small, it is hard to form a bright image with excellent brightness and concealability. When this ratio is excessively increased, the brightness of the bright image may be decreased.

<Method for Producing First and Second Toners>

The first and second toners are produced by, for example, the following method. That is, each of the first and second toners is produced by, for example, a method including a step of producing first and second toner particles through a resin pulverization liquid preparation step S10, a wax pulverization liquid preparation step S11, a toner composition aggregate dispersion liquid preparation step S12, and a toner particle drying step S13, and also including an external additive attaching step S14.

<Resin Pulverization Liquid Preparation Step S10>

In the resin pulverization liquid preparation step S10, a mixed liquid in which a binder resin, a surfactant, a pH adjusting agent, and water are mixed is prepared, followed by mechanical shearing.

The surfactant is not particularly limited, however, for example, an anionic surfactant such as a sulfate ester salt-based, sulfonate salt-based, phosphate ester salt-based, or fatty acid salt-based anionic surfactant, a cationic surfactant such as an amine salt-based or quaternary ammonium salt-based cationic surfactant, an amphoteric surfactant such as a betaine-based amphoteric surfactant, a nonionic surfactant such as a polyethylene glycol-based, alkyl phenol ethylene oxide adduct-based, or polyhydric alcohol-based nonionic surfactant, or a polymeric surfactant such as a polycarboxylic acid can be used. The further incorporation of the surfactant in the first and second toner particles is advantageous for enhancing the stability of the aggregated particles or the dispersion stability thereof. Further, when surfactants having opposite polarities are used simultaneously, these surfactants can have a function as an aggregating agent which will be described later. The surfactant may be omitted. When the surfactant is used, the amount thereof is appropriately set according to the formulation and materials.

The pH adjusting agent is not particularly limited, however, for example, a basic compound such as sodium hydroxide, potassium hydroxide, or an amine compound, or an acidic compound such as hydrochloric acid, nitric acid, or sulfuric acid can be used. The pH adjusting agent may be omitted. When the pH adjusting agent is used, the amount thereof is appropriately set according to the formulation and materials.

Further, a zeta-potential adjusting agent may be used. The zeta-potential adjusting agent is not particularly limited, however, a surfactant having an opposite polarity described above, a pH adjusting agent, or the like can be used. According to one example, to a dispersion having a negative

zeta potential, a cationic surfactant is added. This is advantageous for reversing the zeta potential of the dispersion to positive. According to another example, to a dispersion having a positive zeta potential, an anionic surfactant is added. This is advantageous for reversing the zeta potential of the dispersion to negative. According to still another example, to a dispersion of an amphoteric compound, a pH adjusting agent is added to adjust the pH value. This is advantageous for adjusting the positive or negative of the dispersion. The zeta-potential adjusting agent may be omitted. When the zeta-potential adjusting agent is used, the amount thereof is appropriately set according to the formulation and materials.

<Wax Pulverization Liquid Preparation Step S11>

In the wax pulverization liquid preparation step S11, a mixed liquid in which a release agent, a surfactant, a pH adjusting agent, and water are mixed is prepared, followed by mechanical shearing.

As the surfactant and the pH adjusting agent, those described above can be used.

<Toner Composition Aggregate Dispersion Liquid Preparation Step S12>

In the toner composition aggregate dispersion liquid preparation step S12, first, a resin-wax mixed liquid in which the resin pulverization liquid obtained by the resin pulverization liquid preparation step S10 and the wax pulverization liquid obtained by the wax pulverization liquid preparation step S11 are mixed is prepared. Then, aside from this, a pigment dispersion liquid in which an aggregating agent is added to a mixed liquid of the bright pigment and water is prepared. Subsequently, while stirring the pigment dispersion liquid, the resin-wax mixed liquid is gradually added thereto, whereby a toner composition aggregate dispersion liquid is prepared.

The aggregating agent is not particularly limited, however, a monovalent metal salt such as sodium chloride, a polyvalent metal salt such as magnesium sulfate or aluminum sulfate, a nonmetal salt such as ammonium chloride or ammonium sulfate, an acid such as hydrochloric acid or nitric acid, or a strong cationic coagulating agent such as a polyamine or polydiallyldimethylammonium chloride (polyDADMAC) based coagulating agent can be used. The aggregating agent may be omitted. When the aggregating agent is used, the amount thereof is appropriately set according to the formulation and materials.

<Toner Particle Drying Step S13>

In the toner particle drying step S13, the toner particles are washed and dried.

<External Additive Attaching Step S14>

Finally, in the external additive attaching step S14, an external additive is externally added to the dry toner particles. In the external additive attaching step S14, resin fine particles or inorganic fine particles, or both are externally added and mixed. By doing this, the first toner and the second toner are obtained. The external additive attaching step S14 may be performed after a step of mixing the first toner particles and the second toner particles.

<Step of Mixing First Toner and Second Toner>

In the step of mixing the first toner and the second toner, the first and second toners are mixed as follows. That is, the first and second toners are mixed in such amounts that the ratio of the amount of the second toner to the total amount of the first and the second toners is within the range of 30 to 90 mass %, preferably within the range of 45 to 75 mass %, more preferably within the range of 40 to 70 mass %.

## Other Toners

In the toner cartridges other than the toner cartridge in which the above-mentioned bright toner (hereinafter referred to as "toner A") are stored among the toner cartridges **67Y**, **67M**, **67C**, and **67K**, toners B to D which are different from the toner A may be stored.

For example, as the toners B to D, bright toners which exhibit colors different from the toner A may be used. As such bright toners, for example, those described for the toner A can be used.

When bright toners are used as the toners B to D, the volume particle diameter distributions of the toners B to D are preferably in the same manner as that of the toner A.

Alternatively, as the toners B to D, non-bright toners which exhibit the same color or different colors may be used. When non-bright toners are used as the toners B to D, the volume particle diameter distribution of the toner is not particularly limited. In the non-bright toner, for example, the following colorant can be used.

As the colorant to be contained in the toners B to D, for example, a carbon black can be used. As the carbon black, for example, acetylene black, furnace black, thermal black, channel black, or Ketjen black can be used.

As the colorant to be contained in the toners B to D, a pigment or a dye composed of an organic substance or an inorganic substance may be used. As the pigment or dye, for example, fast yellow G, benzidine yellow, indofast orange, irgaj in red, carmen FB, permanent bordeaux FRR, pigment orange R, lithol red 2G, lake red C, rhodamine FB, rhodamine B lake, phthalocyanine blue, pigment blue, brilliant green B, phthalocyanine green, or quinacridone can be used. As the colorant, among these, one type may be used alone or a mixture of two or more types may be used.

## &lt;&lt;Image Forming Method&gt;&gt;

Next, an image forming method according to an embodiment will be described.

Hereinafter, as one example, an image forming method using the image forming apparatus 1 described with reference to FIGS. 1 to 3 will be described.

First, for example, an operator inputs the information of an image including a portion to be formed with a toner containing a bright pigment (hereinafter referred to as "bright toner") to the image information input section 100 through a network or from an external recording medium. This image may be composed of only a portion to be formed with the bright toner, or may include a first portion to be formed with the bright toner and a second portion to be formed with a toner containing a non-bright pigment (hereinafter referred to as "non-bright toner"). Here, as one example, it is assumed that the above image includes the first and second portions, and the developer in the toner cartridge **67Y** contains the toner A which is the bright toner, and the developers in the toner cartridges **67M**, **67C**, and **67K** each contain the non-bright toner.

The image information input section 100 outputs this image information to the control section 200. The control section 200 controls the operation of the paper feed section 10, the optical unit 20, the image forming section 50, the fixing section 70, the carrying section 80, etc. based on this image information as follows.

First, the control section 200 controls the operation of the paper feed section 10 so that one pickup roller 12 feeds a sheet P which is the top layer among the sheets stored in the paper feed cassette 11 corresponding to this pickup roller 12 to the resist roller 81.

Further, the control section 200 controls the optical unit 20 and the image forming section 50 so that these members perform the following operations.

The secondary transfer roller 54 which is a drive roller 5 rotates the intermediate transfer belt 51 in the counterclockwise direction in FIG. 11. The photoconductors **61Y**, **61M**, **61C**, and **61K** rotate in the clockwise direction in FIG. 1. The chargers **62Y**, **62M**, **62C**, and **62K** uniformly charge the surfaces of the photoconductors **61Y**, **61M**, **61C**, and **61K**, respectively. The optical unit 20 forms a first electrostatic latent image corresponding to the first portion on the surface of the photoconductor **61Y**, forms a second electrostatic latent image corresponding to a part of the second portion on the surface of the photoconductor **61M**, forms a third electrostatic latent image corresponding to another part of the second portion on the surface of the photoconductor **61C**, and forms a fourth electrostatic latent image corresponding to the rest of the second portion on the surface of the photoconductor **61K**.

The developing device **63Y** forms a first toner image corresponding to the first electrostatic latent image on the surface of the photoconductor **61Y**. The developing device **63M** forms a second toner image corresponding to the second electrostatic latent image on the surface of the photoconductor **61M**. The developing device **63C** forms a third toner image corresponding to the third electrostatic latent image on the surface of the photoconductor **61C**. The developing device **63K** forms a fourth toner image corresponding to the fourth electrostatic latent image on the surface of the photoconductor **61K**. The primary transfer rollers **64Y**, **64M**, **64C**, and **64K** transfer the above toner images onto the intermediate transfer belt 51 from the photoconductors **61Y**, **61M**, **61C**, and **61K**, respectively.

The control section 200 controls the operation of the optical unit 20 and the image forming section 50 such that the first toner image is located on a first region corresponding to the first portion, the second toner image is located on a part of a second region corresponding to the second portion, the third toner image is located on another part of the second region, and the fourth toner image is located on the rest of the second region on the surface of the intermediate transfer belt 51. The first toner image forms a bright image.

Further, the control section 200 controls the operation of the image forming section 50 and the carrying section 80 so that when a portion corresponding to the first and second regions of the intermediate transfer belt 51 passes through the secondary transfer roller 54, the sheet P passes between the intermediate transfer belt 51 and the backup roller 55, and at this time, the first to fourth toner images on the intermediate transfer belt 51 are transferred onto the sheet P.

Thereafter, the control section 200 controls the operation of the fixing section 70 and the carrying section 80 so that the first to fourth toner images are fixed to the sheet P, and then, the sheet P is discharged to the paper discharge tray 84. As described above, a printed material including a bright image and a non-bright image is obtained.

## &lt;&lt;Effect&gt;&gt;

When a bright toner having a large particle diameter is used, excellent brightness is expected to be exhibited. However, when an image is formed on the sheet P using only such a bright toner, inconvenience is likely to occur in development or transfer, and therefore, a gap is likely to occur in a portion where the bright toners are superimposed on each other on the sheet P. That is, in this case, there is still room for improvement on the concealability.

Further, when an image is formed on the sheet P using a bright toner having a small particle diameter, excellent concealability is expected. However, when only such a bright toner is used, also the particle diameter of the bright pigment is small, and therefore, high brightness as in the case where only a bright toner having a larger particle diameter is used cannot be achieved.

On the other hand, in the process described with reference to FIGS. 1 to 3, the bright toner in which the particle size distribution is optimized by mixing the first and second toners having different volume average particle diameters is used in the formation of a bright image. Therefore, excellent brightness and excellent concealability can be achieved simultaneously.

The above-mentioned image forming apparatus 1 includes the intermediate transfer belt 51, however, the image forming apparatus 1 may be an image forming apparatus which adopts a direct transfer system. Further, in the above-mentioned image forming apparatus 1, four image forming stations 60Y, 60M, 60C, and 60K are arranged, however, only one image forming station may be provided. In this case, for example, a plurality of developing devices are arranged around one photoconductor.

Further, in the above-mentioned image forming apparatus 1, the toner cartridges 67Y, 67M, 67C, and 67K are detachably placed above the hoppers 66Y, 66M, 66C, and 66K, however, the following form may be adopted. For example, the image forming apparatus 1 may include the toner cartridges 67Y, 67M, 67C, and 67K integrally with the developing devices 63Y, 63M, 63C, and 63K, respectively, and may detachably include this unit. According to another example, the image forming apparatus 1 may include the toner cartridges 67Y, 67M, 67C, and 67K integrally with the developing devices 63Y, 63M, 63C, and 63K, respectively, and also with the photoconductors 61Y, 61M, 61C, and 61K, respectively, and may detachably include this unit.

## EXAMPLES

Hereinafter, specific examples of the embodiments will be described.

### (Production of Toner T1)

A toner T1 was produced by the following method.

First, a resin pulverization liquid was prepared. That is, 30 parts by mass of a polyester-based resin as a binder resin, 3 parts by mass of sodium dodecylbenzenesulfonate as an anionic surfactant, 1 part by mass of triethylamine as a pH adjusting agent, and 66 parts by mass of water were mixed at room temperature. Thereafter, the temperature of the mixed liquid was increased to 80° C., and the mixed liquid was subjected to mechanical shearing for 30 minutes. Specifically, CLEARMIX (registered trademark) was used as a dispersion emulsification machine, and the mechanical shearing was performed by setting the rotation speed of the machine to 6000 rpm. After completion of the mechanical shearing, the temperature of the mixed liquid was decreased to normal temperature.

The volume average particle diameter of the particles included in the obtained resin pulverization liquid was measured by a laser diffraction scattering method. In the measurement performed here, and in the measurement of a volume average particle diameter by a laser diffraction scattering method described below, SALD-7000 (Shimadzu Corporation) was used. As a result, the volume average particle diameter was 0.16  $\mu\text{m}$ .

Subsequently, a wax pulverization liquid was prepared. That is, 40 parts by mass of an ester wax as a release agent,

4 parts by mass of sodium dodecylbenzenesulfonate as an anionic surfactant, 1 part by mass of triethylamine as a pH adjusting agent, and 55 parts by mass of water were mixed at room temperature. Thereafter, the temperature of the mixed liquid was increased to 80° C., and the mixed liquid was subjected to mechanical shearing for 30 minutes by setting the rotation speed of the dispersion emulsification machine to 6000 rpm. After completion of the mechanical shearing, the temperature of the mixed liquid was decreased to normal temperature.

The volume average particle diameter of the obtained wax pulverization liquid was measured by a laser diffraction scattering method. As a result, the volume average particle diameter was 0.20  $\mu\text{m}$ .

50 Parts by mass of the resin pulverization liquid, 8 parts by mass of the wax pulverization liquid, and 42 parts by mass of water were placed in a flask, followed by stirring, whereby a resin-wax mixed liquid was prepared.

Subsequently, a pigment dispersion liquid was prepared by the following method.

First, 31 parts by mass of Iridin 325 as a bright pigment and 589 parts by mass of water were stirred at a stirring speed of 700 rpm at room temperature. The stirring under such conditions was maintained until the below-mentioned toner particle dispersion liquid was obtained.

Subsequently, 25 parts by mass of a 0.5% polydiallyldimethylammonium chloride solution as an aggregating agent was added to this mixed liquid. Then, the temperature of the mixed liquid was increased to 45° C. Subsequently, 50 parts by mass of an aqueous 30% ammonium sulfate solution as an aggregating agent was added to this mixed liquid. Then, stirring was continued for 1 hour while maintaining the temperature and the stirring speed under the above-mentioned conditions. By doing this, a pigment dispersion liquid was obtained.

Subsequently, 250 parts by mass of the resin-wax mixed liquid described above was added to the pigment dispersion liquid from the upper side thereof at a rate of 0.5 parts by mass/min. The addition of the resin-wax mixed liquid was performed using a liquid feed pump capable of controlling the flow rate of the mixed liquid to be added, here, a Masterflex tubing pump system (Yamato Scientific Co., Ltd., inner diameter of tube: 0.8 mm). By doing this, the bright pigment particles were coated with the binder resin and the release agent.

Further, 26 parts by mass of an aqueous 30% ammonium sulfate solution as an aggregating agent was added to this mixed liquid. Then, a mixed liquid composed of 80 parts by mass of the resin pulverization liquid and 80 parts by mass of water was added to the mixed liquid from the upper side thereof at a rate of 0.5 parts by mass/min using the liquid feed pump. By doing this, a toner composition aggregate dispersion liquid was obtained.

Subsequently, to this toner composition aggregate dispersion liquid, 10 parts by mass of a polycarboxylic acid-based surfactant (POIZ (registered trademark) 520, Kao Corporation) was added as a surfactant, and the temperature of the dispersion liquid was increased to 65° C., whereby the particles were partially fused. By doing this, a toner particle dispersion liquid was obtained.

Subsequently, the toner particle dispersion liquid was washed and dried. Specifically, filtration of the toner particle dispersion liquid and washing with water were repeatedly performed until the electrical conductivity of the filtrate was decreased to 50  $\mu\text{S}/\text{cm}$  or less. Thereafter, the toner particles were dried using a vacuum dryer until the water content therein was decreased to 1.0 mass % or less.

## 15

Finally, 2 parts by mass of hydrophobic silica and 0.5 parts by mass of titanium oxide as external additives were added with respect to 100 parts by mass of the dry toner particles and externally added thereto using a Henschel (registered trademark) mixer as a mixing machine, whereby a toner T1 was obtained. The volume average particle diameter of the toner T1 was measured by an electrical sensing zone method. In the measurement performed here, and in the measurement of the volume average particle diameter by an electrical sensing zone method described below, Multisizer 3 (Coulter Counter) was used. As a result, the volume average particle diameter was 13.23  $\mu\text{m}$ .

## (Production of Toner T2)

A toner T2 was obtained in the same manner as the method for producing the toner T1 except that the pigment was changed from Iridin 325 to Iridin 305. The volume average particle diameter of the toner T2 was 19.72  $\mu\text{m}$ .

## (Production of Toner T3)

A toner T3 was obtained in the same manner as the method for producing the toner T1 except that the stirring speed in the preparation of the pigment dispersion liquid and the subsequent step was changed from 700 rpm to 800 rpm. The volume average particle diameter of the toner T3 was 12.52  $\mu\text{m}$ .

## (Production of Toner T4)

A toner T4 was obtained in the same manner as the method for producing the toner T2 except that the stirring speed in the preparation of the pigment dispersion liquid and the subsequent step was changed from 700 rpm to 800 rpm. The volume average particle diameter of the toner T4 was 18.87  $\mu\text{m}$ .

## (Production of Toner T5)

A toner T5 was obtained in the same manner as the method for producing the toner T1 except that the stirring speed in the preparation of the pigment dispersion liquid and the subsequent step was changed from 700 rpm to 500 rpm. The volume average particle diameter of the toner T5 was 15.23  $\mu\text{m}$ .

By using the toners T1 to T5 obtained by the above-mentioned methods, image formation was performed as follows. Here, image formation was performed using the image forming apparatus 1 described with reference to FIGS. 1 to 3.

## Example 1

Image formation was performed using a bright toner E1 obtained by mixing 80 parts by mass of the toner T2 and 20 parts by mass of the toner T1. The volume average particle diameter of the bright toner E1 was 17.83  $\mu\text{m}$  and the coefficient of variation CV was 0.27.

In the toner cartridge body 671K, a two-component developer containing the bright toner E1 and a ferrite carrier was filled. In this two-component developer, the ratio of the mass of the bright toner E1 to the mass of the ferrite carrier (toner ratio concentration) was 8%.

By the method described with reference to FIGS. 1 to 3, a bright solid patch image was formed on a sheet P in a normal temperature and normal humidity environment. Here, as the image forming apparatus 1, an electrophotographic MFP (e-studio 4520c, Toshiba Tec Corporation) was used. Further, the total amount of the bright toner attached in a region where the image was formed in the recording medium was set to 0.50 mg/cm<sup>2</sup>. The ratio of the volume

## 16

average particle diameter of the toner T2 to the volume average particle diameter of the toner T1 was 1.49.

## Example 2

Image formation was performed in the same manner as in Example 1 except that a bright toner E2 obtained by mixing 40 parts by mass of the toner T2 and 60 parts by mass of the toner T1 was used. The volume average particle diameter of the bright toner E2 was 15.89  $\mu\text{m}$  and the coefficient of variation CV was 0.29.

## Example 3

Image formation was performed in the same manner as in Example 1 except that a bright toner E3 obtained by mixing 85 parts by mass of the toner T2 and 15 parts by mass of the toner T1 was used. The volume average particle diameter of the bright toner E3 was 18.01  $\mu\text{m}$  and the coefficient of variation CV was 0.26.

## Example 4

Image formation was performed in the same manner as in Example 1 except that a bright toner E4 obtained by mixing 60 parts by mass of the toner T4 and 40 parts by mass of the toner T3 was used. The ratio of the volume average particle diameter of the toner T4 to the volume average particle diameter of the toner T3 was 1.51. The volume average particle diameter of the bright toner E4 was 15.72  $\mu\text{m}$  and the coefficient of variation CV was 0.27.

## Example 5

Image formation was performed in the same manner as in Example 1 except that a bright toner E5 obtained by mixing 60 parts by mass of the toner T2 and 40 parts by mass of the toner T1 was used. The volume average particle diameter of the bright toner E5 was 16.53  $\mu\text{m}$  and the coefficient of variation CV was 0.29.

## Example 6

Image formation was performed in the same manner as in Example 1 except that a bright toner E6 obtained by mixing 70 parts by mass of the toner T2 and 30 parts by mass of the toner T1 was used. The volume average particle diameter of the bright toner E6 was 17.24  $\mu\text{m}$  and the coefficient of variation CV was 0.28.

## Example 7

Image formation was performed in the same manner as in Example 1 except that a bright toner E7 obtained by mixing 50 parts by mass of the toner T2 and 50 parts by mass of the toner T1 was used. The volume average particle diameter of the bright toner E7 was 16.16  $\mu\text{m}$  and the coefficient of variation CV was 0.29.

## Example 8

Image formation was performed in the same manner as in Example 1 except that a bright toner E8 obtained by mixing 60 parts by mass of the toner T4 and 40 parts by mass of the toner T5 was used. The ratio of the volume average particle diameter of the toner particles included in the toner T4 to the volume average particle diameter of the toner particles included in the toner T5 was 1.24. The volume average particle diameter of the bright toner E8 was 17.21  $\mu\text{m}$  and the coefficient of variation CV was 0.27.

## Comparative Example 1

Image formation was performed in the same manner as in Example 1 except that a bright toner C1 composed of only the toner T2 was used. The volume average particle diameter of the bright toner C1 was 19.72  $\mu\text{m}$  and the coefficient of variation CV was 0.24.

## Comparative Example 2

Image formation was performed in the same manner as in Example 1 except that a bright toner C2 obtained by mixing

50 parts by mass of the toner T2 and 50 parts by mass of the toner T4 was used. The ratio of the volume average particle diameter of the toner T2 to the volume average particle diameter of the toner T4 was 1.05. The volume average particle diameter of the bright toner C5 was 19.28  $\mu\text{m}$  and the coefficient of variation CV was 0.25.

## &lt;Evaluation&gt;

10 With respect to the images formed in Examples 1 to 8 and Comparative Examples 1 to 5, brightness and concealability were evaluated. The results are shown in Table 1.

TABLE 1

|                       | Bright toner |                                             |                  |              |                                         |                                   |          |            |                |
|-----------------------|--------------|---------------------------------------------|------------------|--------------|-----------------------------------------|-----------------------------------|----------|------------|----------------|
|                       | CV value     | Average particle diameter ( $\mu\text{m}$ ) | Ratio of average |              | Ratio of second toner particle diameter | Bright pigment particles (mass %) | CV value | Brightness | Concealability |
|                       |              |                                             | First toner      | Second toner |                                         |                                   |          |            |                |
| Example 1             | 0.27         | 17.83                                       | T1               | T2           | 1.49                                    | 80                                | 0.42     | B          | A              |
| Example 2             | 0.29         | 15.89                                       | T1               | T2           | 1.49                                    | 40                                | 0.49     | A          | B              |
| Example 3             | 0.26         | 18.01                                       | T1               | T2           | 1.49                                    | 85                                | 0.50     | B          | A              |
| Example 4             | 0.27         | 15.72                                       | T3               | T4           | 1.51                                    | 60                                | 0.45     | B          | A              |
| Example 5             | 0.29         | 16.53                                       | T1               | T2           | 1.49                                    | 60                                | 0.45     | A          | A              |
| Example 6             | 0.28         | 17.24                                       | T1               | T2           | 1.49                                    | 70                                | 0.41     | A          | A              |
| Example 7             | 0.29         | 16.16                                       | T1               | T2           | 1.49                                    | 50                                | 0.47     | A          | A              |
| Example 8             | 0.27         | 17.21                                       | T5               | T4           | 1.24                                    | 60                                | 0.47     | A          | A              |
| Comparative Example 1 | 0.24         | 19.72                                       | —                | T2           | —                                       | —                                 | 0.40     | A          | C              |
| Comparative Example 2 | 0.25         | 15.71                                       | T1               | T2           | 1.49                                    | 20                                | 0.50     | C          | B              |
| Comparative Example 3 | 0.25         | 14.58                                       | T3               | T4           | 1.51                                    | 20                                | 0.50     | C          | B              |
| Comparative Example 4 | 0.25         | 12.93                                       | T3               | T1           | 1.06                                    | 50                                | 0.46     | C          | A              |
| Comparative Example 5 | 0.25         | 19.28                                       | T4               | T2           | 1.05                                    | 50                                | 0.45     | A          | C              |

20 parts by mass of the toner T2 and 80 parts by mass of the toner T1 was used. The volume average particle diameter of the bright toner C2 was 15.71  $\mu\text{m}$  and the coefficient of variation CV was 0.25.

## Comparative Example 3

Image formation was performed in the same manner as in Example 1 except that a bright toner C3 obtained by mixing 20 parts by mass of the toner T4 and 80 parts by mass of the toner T3 was used. The volume average particle diameter of the bright toner C3 was 14.58  $\mu\text{m}$  and the coefficient of variation CV was 0.25.

## Comparative Example 4

Image formation was performed in the same manner as in Example 1 except that a bright toner C4 obtained by mixing 50 parts by mass of the toner T1 and 50 parts by mass of the toner T3 was used. The ratio of the volume average particle diameter of the toner T1 to the volume average particle diameter of the toner T3 was 1.06. The volume average particle diameter of the bright toner C4 was 12.93  $\mu\text{m}$  and the coefficient of variation CV was 0.25.

## Comparative Example 5

Image formation was performed in the same manner as in Example 1 except that a bright toner C5 obtained by mixing

## 40 (Evaluation of Brightness)

The obtained images were observed, and the brightness thereof was evaluated by visual observation. Here, the observation was performed under the conditions of "Illuminant A" of SpectraLight QC (X-Rite, Inc.). In Table 1, a sample which could be confirmed to have sufficient brightness when the sample was placed on a table and observed from an angle of 45° and 60° is shown as "A", a sample which could be confirmed to have brightness only when the sample was held by hand and observed from different angles is shown as "B", and a sample which could be confirmed to have low brightness only when a test image was held by hand and observed from different angles in a state where the sample was further irradiated with the light of a fluorescent lamp is shown as "C".

## 45 (Evaluation of Concealability)

With respect to the samples used for the evaluation of brightness, observation and image acquisition were performed using an optical microscope.

A lens with a magnification of 10 $\times$  was used as an ocular lens, and a lens with a magnification of 10 $\times$  was used as an objective lens. Then, by using an image analysis software ImageJ, the area ratio of a bright pigment portion to the entire printed image region was determined from the obtained image.

50 In Table 1, a sample in which the area ratio of a bright pigment portion was 60% or more is shown as "A", a sample in which the area ratio of a bright pigment portion was 50%

19

or more and less than 60% is shown as "B", and a sample in which the area ratio of a bright pigment portion was less than 50% is shown as "C".

As shown in Table 1, in Examples 1 to 8, excellent brightness and concealability were achieved as compared with Comparative Examples 1 to 5.

Further, in Examples 5 to 8, particularly excellent brightness and concealability were achieved.

The measurement of the volume particle diameter distribution of the bright pigments contained in the bright toners of Examples 1 to 8 and Comparative Examples 1 to 5 was performed before production of the toners. Specifically, the bright pigments to be used were prepared, mixed according to the mixing ratio shown in Table 1, and then, the measurement was performed. The coefficient of variation CV of the particle size distribution is shown in Table 1.

As shown in Table 1, the correlation between the coefficient of variation CV of the particle size distribution of the bright pigment and the brightness and concealability was low.

The invention is not limited to the embodiments described above and can be modified variously without departing from the gist of the invention when it is practiced. Also, the respective embodiments may be appropriately combined and carried out, and combined effects can be obtained in this case. Further, the embodiments described above include various inventions, and various inventions can be extracted based on combinations selected from a plurality of disclosed constituent elements. For example, even if several constituent elements are deleted from all the constituent elements disclosed in the embodiments, a structure in which the constituent elements are deleted can be extracted as the invention when the problem can be solved and the effect can be obtained.

What is claimed is:

1. A bright toner comprising a plurality of toner particles containing a bright pigment and a binder resin, and having a volume particle diameter distribution with a coefficient of variation CV of 0.26 or more, wherein the bright pigment has a volume particle size distribution with a coefficient of variation CV of 0.41 to 0.50.

2. The toner according to claim 1, wherein the toner is a mixture comprising:

a first toner which comprises a plurality of first toner particles containing a first bright pigment and a first binder resin, and has a first volume average particle diameter, and

a second toner which comprises a plurality of second toner particles containing a second bright pigment and a second binder resin, and has a second volume average particle diameter, wherein the ratio of the second volume average particle diameter to the first volume average particle diameter is 1.10 or more, wherein the ratio of the amount of the second toner to the total amount of the first toner and the second toner is within the range of 30 to 90 mass %.

3. The toner according to claim 2, wherein the ratio of the second volume average particle diameter to the first volume average particle diameter is 1.20 to 1.50.

4. The toner according to claim 2, wherein the ratio of the amount of the second toner to the total amount of the first toner and the second toner is within the range of 40 to 70 mass %.

5. The toner according to claim 1, wherein the bright pigment exhibits metallic luster or pearly luster.

20

6. The toner according to claim 1, wherein the bright toner has a volume particle diameter distribution with a coefficient of variation CV of 0.30 or less.

7. The toner according to claim 1, wherein the bright toner has a volume particle diameter distribution with a coefficient of variation CV of 0.27 to 0.29.

8. The toner according to claim 1, wherein the volume average particle diameter of the bright toner is 7.0 to 105.0  $\mu\text{m}$ .

9. The toner according to claim 1, wherein the volume average particle diameter of the bright toner is 16.0 to 17.7  $\mu\text{m}$ .

10. An image forming apparatus, comprising:  
a photoconductor;  
a charger which charges the photoconductor;

an optical unit which irradiates the photoconductor with light, thereby forming an electrostatic latent image;  
a developing device comprising the bright toner of claim

1, wherein the developing device supplies the bright toner to the photoconductor, thereby forming a toner image corresponding to the electrostatic latent image; and

a transfer device which directly or indirectly transfers the toner image onto a recording medium from the photoconductor.

11. A bright toner comprising a plurality of toner particles containing a bright pigment and a binder resin, and having a volume particle diameter distribution with a coefficient of variation CV of 0.26 or more, wherein the bright pigment has a number particle size distribution with a coefficient of variation CV of 0.50 to 0.57.

12. The toner according to claim 11, wherein the toner is a mixture comprising:

a first toner which comprises a plurality of first toner particles containing a first bright pigment and a first binder resin, and has a first volume average particle diameter, and

a second toner which comprises a plurality of second toner particles containing a second bright pigment and a second binder resin, and has a second volume average particle diameter, wherein the ratio of the second volume average particle diameter to the first volume average particle diameter is 1.10 or more,

wherein the ratio of the amount of the second toner to the total amount of the first toner and the second toner is within the range of 30 to 90 mass %.

13. The toner according to claim 12, wherein the ratio of the second volume average particle diameter to the first volume average particle diameter is 1.20 to 1.50.

14. The toner according to claim 12, wherein the ratio of the amount of the second toner to the total amount of the first toner and the second toner is within the range of 40 to 70 mass %.

15. The toner according to claim 11, wherein the bright pigments each exhibits metallic luster or pearly luster.

16. The toner according to claim 11, wherein the bright toner has a volume particle diameter distribution with a coefficient of variation CV of 0.30 or less.

17. The toner according to claim 11, wherein the bright toner has a volume particle diameter distribution with a coefficient of variation CV of 0.27 to 0.29.

18. The toner according to claim 11, wherein the volume average particle diameter of the bright toner is 7.0 to 105.0  $\mu\text{m}$ .

19. The toner according to claim 11, wherein the volume average particle diameter of the bright toner is 16.0 to 17.7  $\mu\text{m}$ .

20. An image forming apparatus, comprising:  
a photoconductor;  
a charger which charges the photoconductor;  
an optical unit which irradiates the photoconductor with  
light, thereby forming an electrostatic latent image; 5  
a developing device comprising the bright toner of claim  
11, wherein the developing device supplies the bright  
toner to the photoconductor, thereby forming a toner  
image corresponding to the electrostatic latent image;  
and 10  
a transfer device which directly or indirectly transfers the  
toner image onto a recording medium from the photo-  
conductor.

\* \* \* \* \*